

# UNITED STATES PATENT OFFICE.

VOLNEY E. BROWN, OF WOODSTOCK, ILLINOIS.

## COMPOSITION FOR CLEANING METALS.

SPECIFICATION forming part of Letters Patent No. 697,976, dated April 22, 1902.

Application filed September 25, 1901. Serial No. 76,567. (No specimens.)

*To all whom it may concern:*

Be it known that I, VOLNEY E. BROWN, a citizen of the United States, residing at Woodstock, in the county of McHenry and State of Illinois, have invented certain new and useful Improvements in Compounds for Polishing Metal, of which the following is a specification.

The object of my invention is to provide an improved compound for polishing metals.

In carrying out my invention I combine the following ingredients in about the following proportions: cake-tallow, one and one-fourth pounds; gum-camphor, three ounces; beeswax, four ounces; raw linseed - oil, eight ounces; kerosene - oil, fifteen ounces; powdered tripoli, two pounds; oil of spearmint, one ounce. In mixing these ingredients the cake-tallow, gum-camphor, and beeswax are first melted together, and as soon as they are melted the raw linseed-oil is poured in. Then the kerosene is added, and while this mixture is still hot the powdered tripoli is added. This mixture is allowed to cool until it starts to get thick, and then the spearmint is added to give it a pleasant odor. The result is a

pasty compound, which is put up for the market in cans, bottles, or boxes. The compound is applied by rubbing it on the metal by means of a soft rag.

The relative proportions may be slightly varied without departing from my invention. The oil of spearmint is employed to give the compound a pleasant odor. Any other suitable perfume may be used in place of the spearmint.

I claim as my invention—

A metal-polishing compound consisting of the following ingredients in substantially the following proportions: cake-tallow, one and one - fourth pounds; gum - camphor, three ounces; beeswax, four ounces; raw linseed-oil, eight ounces; kerosene-oil, fifteen ounces; powdered tripoli, two pounds, and a suitable quantity of perfume.

In testimony whereof I have hereunto subscribed my name.

V. E. BROWN.

Witnesses:

A. S. WRIGHT, Jr.  
D. T. SMILEY.